

# UNITED STATES PATENT OFFICE.

JOSEPH HAY AMIES, OF PHILADELPHIA, PENNSYLVANIA, ASSIGNOR TO THE AMIES ASPHALT COMPANY, OF PHILADELPHIA, PENNSYLVANIA, A CORPORATION OF SOUTH DAKOTA.

## ROAD AND STREET SURFACING.

1,082,478.

No Drawing.

Specification of Letters Patent.

Patented Dec. 23, 1913.

Application filed March 7, 1913. Serial No. 752,586.

To all whom it may concern:

Be it known that I, JOSEPH HAY AMIES, a citizen of the United States, residing at Philadelphia, in the county of Philadelphia and State of Pennsylvania, have invented 5 certain new and useful Improvements in Road and Street Surfacing, of which the following is a specification.

This invention has relation to road and 10 street construction wherein Portland cement concrete or grout or mortar is employed to which is added a bituminous facing and the principal object of the present invention is to provide a facing for concrete or like paving 15 in which hydrocarbon or carbonaceous oils are treated to prevent their oxidation by practically fixing them by causing them to become albuminized.

A further object of the invention is to 20 provide a novel, efficient and inexpensive bituminous facing for concrete or like paving which may be easily and expeditiously laid.

A still further object of the invention is 25 to apply to such concrete or like road or street a facing containing hydrocarbon or carbonaceous oil calculated to take up the inherent moisture present in the concrete in order to secure a good bond.

30 With these and other objects in view the invention consists of the improvements hereinafter described and finally claimed.

In the practice of the invention, the road or street is constructed according to standard methods employing Portland cement or 35 grout or mortar and mineral or earthy materials and water as may be called for by the specifications followed. After the setting of the concrete or like paving, I apply 40 the facing of the invention, which, it may be stated, can be applied under varying climatic conditions. The facing is prepared as follows: I first add to calcium oxid in a powdered condition, boiling water in order 45 to render the calcium oxid a stiff mortar-like mass. The hot water will cause the calcium oxid to immediately slake at which time I thoroughly mix therewith a highly heated hydrocarbon or carbonaceous oil. 50 Such hydrocarbon or carbonaceous oil must be of a desirable penetration and should be heated to about 320 degrees F. During the mixing of the calcium oxid and the heated oil, a violent fomentation takes place and the

oil, due to the escaping vapor given off by the slaking calcium oxid, will expand to a great degree. During the above described fomentation, I spread the thoroughly mixed oil and calcium oxid, at a desired thickness, over the surface of the concrete or like road or street. As is well known, the surface of concrete is naturally cold and damp and inasmuch as the calcium oxid of the above described mixture has not been provided with sufficient water to gratify it, said calcium oxid will, by chemical affinity, take up the inherent moisture of the concrete surface and warm the same sufficiently by the heat generated by the calcium oxid to cause the hydrocarbon or carbonaceous oil used to penetrate the concrete. This penetration of the oil is uniform over the concrete surface and in fact affixes itself firmly thereto in a manner calculated to overcome many difficulties and objections heretofore encountered in facing Portland cement concrete and like pavings, with hydrocarbon or carbonaceous oils. I now spread over the concrete or like paving, coated as above described, earthy or mineral materials, preferably hot, which 80 materials are then rolled thereby causing the oil of the coating to ooze up as it were in and through the earthy or mineral materials. The rolling process is continued until a finished wearing surface for the concrete road 85 or street has been effected.

Having thus described the nature and objects of the invention, what I claim is:

1. The herein described method of treating the surface of a concrete, grout or mortar or like road or street which consists in first spreading over the surface thereof a mixture of heated hydrocarbon or carbonaceous oil, calcium oxid and hot water which mixture is applied while the calcium oxid is slaking and in a condition of active fomentation, then spreading thereover heated earthy or mineral materials and finally subjecting the same to compression to form a wearing surface. 90

2. The herein described method of treating the surface of a concrete, grout, mortar or like street or road which consists in first spreading over the surface thereof a mixture of hydrocarbon or carbonaceous oil, 95 calcium oxid and hot water which mixture is applied while the calcium oxid is slaking and in a condition of active fomentation 100

105

which slaking of the calcium oxid serves to take up the inherent moisture of the paving and causes the same to readily accept and permit the penetration of said oil, then spreading thereover heated earthy or mineral materials and finally subjecting the same to compression to form a wearing surface said compression causing said oil to

ooze up into and through said earthy and mineral materials.

In testimony whereof, I have hereunto signed my name.

JOSEPH HAY AMIES.

Witnesses:

WILLIAM J. JACKSON,  
AGNES E. CASKEY.